

July 5, 1960

L. B. TAYLOR

2,943,971

PIGMENTED PAPER AND PREPARATION THEREOF

Original Filed Oct. 31, 1955



FIG. 2



FIG. 1

INVENTOR.  
LOUIS B. TAYLOR

Oscar H. Spencer  
ATTORNEY

1

2,943,971

## PIGMENTED PAPER AND PREPARATION THEREOF

Louis B. Taylor, Pittsburgh, Pa., assignor to Columbia-Southern Chemical Corporation, Allegheny County, Pa., a corporation of Delaware

Continuation of application Ser. No. 543,835, Oct. 31, 1955. This application July 31, 1959, Ser. No. 830,859

13 Claims. (Cl. 162—181)

The present invention deals with pigmented paper and the manufacture thereof, and more particularly involves enhancing the opacity, brightness and other desirable properties of paper by pigmentation with titanium dioxide and finely divided, amorphous siliceous materials.

Heretofore, various proposals have been offered for improving paper quality, especially with printing papers, by pigmentation with materials, one of the most noteworthy of which is titanium dioxide. Due to its high cost, titanium dioxide is not economically suitable for all grades of paper but finds favor in only the more expensive papers. Also, the retention of titanium dioxide in paper during the paper sheeting step leaves room for betterment. Among other things, the recovery and recirculation of unretained titanium dioxide in the white waters is cumbersome and inefficient.

According to the present invention, the disadvantage and high costs which accompany titanium dioxide pigmentation are minimized and/or obviated. It is possible to reduce the required quantity of titanium dioxide, and consequently the cost of pigmentation, while not sacrificing paper quality. Instead, paper of improved opacity and brightness is obtained. Further realized is increased pigment retention in the paper sheeting step.

Now it has been discovered that such benefits ensue from sheeting a pulp slurry which includes both titanium dioxide and a finely divided, amorphous siliceous pigmentary material, notably calcium silicate. Viewed otherwise, it has been found that up to 90 weight percent of titanium dioxide normally required for a given pigmentation may be replaced with finely divided, amorphous siliceous pigments of much less cost. As a consequence, costs are reduced and a pigmented paper is prepared which has high opacity, brightness and increased quantities of pigment. Often these paper qualities are superior to those which can be obtained using either titanium dioxide or the siliceous material individually.

Figures I and II in the drawing pictorially demonstrate the synergistic effects observed in connection with the practice of this invention. Thus, in Figure I, the variations in opacity and ash (pigment retained in the paper) for differing ratios of titanium dioxide and calcium silicate are graphically shown. With only titanium dioxide the paper's opacity is about 86.5, yet opacities in excess of this value are achieved with pigmenting materials containing from about 40 percent to about 95 percent titanium dioxide by weight of titanium dioxide and calcium silicate. Furthermore, even with larger percentages of calcium silicate opacities are of values which are in excess of those which might be expected from the contribution thereto of the respective pigments.

In a similar fashion, greatly increased ash contents are observed by practice of this invention. For the given conditions, hereinafter detailed, ashes are of about 6.5 percent with either pigment, yet when using combinations thereof, ashes range substantially above 6.5 percent and as high as about 8.3 percent (when the pigment comprises 80

2

percent titanium dioxide by weight thereof and calcium silicate).

Thus, according to one embodiment, the utilization of calcium silicate or comparable pigmentary siliceous material offers an expedient for increasing the concentration of pigment composition including titanium dioxide in paper. In another embodiment, paper opacities in excess of those possible with titanium dioxide are realized. And in a still further embodiment, the value of calcium silicate or other siliceous material, particularly those of low cost, may be increased as an opacifying agent.

In practice, the advantages of the present invention are realized by recourse to any of a number of procedures. Briefly, both titanium dioxide and the siliceous ingredient, notably finely divided calcium silicate, are added to a pulp slurry most advantageously after the pulp has been beaten suitably following usual paper beating practices. Thereafter, the slurry pH is adjusted to within the range of about 4 to 6.5, notably pH 5, by adding an acidic material such as aluminum sulphate or other sulphuric acid salt including sodium sulphate and sodium bisulphate or sulphuric acid itself. Also, other acidic materials, generally inorganic acids such as hydrochloric acid, carbonic acid, etc. or their anhydrides or acid salts are effective. Aluminum sulphate (alum) finds widest use, not only because it is particularly effective but also because it is a common material used in paper manufacture for other reasons. Because of its low cost, sulphuric acid is an excellent replacement for part or all of the alum. This acidified slurry is sheeted into paper on recognized apparatus, e.g. a Fourdrinier or cylinder machine.

Sometimes, after including the pigments in the pulp slurry, even following substantial beating, the dispersion of the pigments is enhanced by further agitation of the pulp slurry as by mechanical stirring or even beating. This facilitates uniform distribution of the pigment throughout the slurry.

Depending to some extent upon the exact paper employed, the particular quality of paper desired, and other peculiarities of any given paper forming operation, the ratio of the two pigments may be varied. Beneficial results are obtained when employing from about 10 to about 95 percent titanium dioxide by weight of titanium dioxide and calcium silicate. With lower titanium dioxide concentrations, the pigmenting qualities of calcium silicate are upgraded strikingly and according to one embodiment hereof, this constitutes an important consideration in utilizing the concepts of this invention. Thus, when papers of opacities slightly higher than are otherwise attained with calcium silicate or comparable siliceous material are the object, a minor quantity of titanium dioxide suffices.

However, in a preferred embodiment, the titanium dioxide is employed in quantities ranging from about 35 or 40 percent to about 95 percent by weight thereof and calcium silicate. Opacities exceeding those of titanium dioxide pigmented papers are realized within this range, see Figure I of the drawing and Example I hereinafter.

With certain pulps, the contribution to opacity and other paper characteristics by both the combination of titanium dioxide and calcium silicate appears even more noticeable, note Example II hereinafter and Figure II of the drawings. There, paper prepared from a pulp furnish consisting solely of kraft pulp to which had been added both pigmentary materials was of superior opacity and brightness by comparison with the values obtained with the individual pigments regardless of the ratio of the titanium dioxide and calcium silicate.

Mixtures of titanium dioxide and calcium silicate, for this invention, may be provided directly in the pulp slurry by addition of requisite quantities of independently pre-

pared pigments to the slurry, or the two may be mixed prior to being added to the slurry.

In the case of siliceous materials, such as the preferred calcium silicate, the pH adjustment of the slurry may include a chemical change. Aluminum sulphate reacts with calcium silicate, probably to provide a calcium aluminum silicate and calcium sulphate, the latter having some water solubility which may, at least in part, account for removal of calcium sulphate in the white waters. Chemical reactions may be encountered with other silicates, notably between alkaline earth metal silicates, and other useful acidic materials which form water insoluble alkaline earth metal salts. For the most part, the acidic material requirements for pH adjustment are less than the stoichiometric quantity needed to react completely with the siliceous pigment. Hence, usually at least a portion of siliceous pigment such as calcium silicate reacts with the acidic material, e.g. aluminum sulphate. Under specialized circumstances the calcium silicate may be completely reacted or decomposed. In many instances, the reaction between the acidic material and siliceous pigment proceeds so slowly that the acidic material is not completely consumed prior to sheeting.

A large variety of finely divided, amorphous pigmentary siliceous materials containing at least about 50 percent  $\text{SiO}_2$  by weight (anhydrous or water free basis) are useful either alone or in combination. Foremost among these are the finely divided, amorphous, pigmentary calcium silicates ranging in surface areas from 10 to 60 square meters per gram, as measured by the Brunauer-Emmett-Teller method described in the Journal of American Chemical Society, volume 60, page 309 (1938) which corresponds to the formula  $\text{CaO}(\text{SiO}_2)_x$ ,  $x$  ranging from about 2 to 5, and particularly from 2.9 to 3.8. Those calcium silicates having packed bulk densities preferably from 0.1 to 0.4 gram per cubic centimeter as measured at three pounds per square inch give pronounced beneficial effects. Such calcium silicates appear to be in the form of flocs of finely divided ultimate calcium silicate particles when viewed under high magnification. Under the electron microscope, the flocs resemble clusters of grapes and appear to be a loosely connected agglomeration of ultimate particles. Their ultimate particle size is below 1.0 micron, usually in the range of 0.015 to 0.2 with the average particle size being from 0.04 to 0.08 micron. The flocs range in size from about 0.6 or 1 micron to as high as 10 microns, the majority thereof, e.g. at least about 55 per cent by weight, being from 1 to 5 microns.

The beneficial effects are not limited to use of the preferred calcium silicates, but may be obtained by recourse to other finely divided, amorphous siliceous materials. Somewhat finer calcium silicates which have BET surface areas ranging upwards of 50 or 60 to from 120 to 200 square meters per gram comprise a useful component. Still other amorphous, finely divided calcium silicates and mixed calcium silicates containing at least about 50 weight percent  $\text{SiO}_2$  and of below 1.0 micron particle size, more preferably below 0.3 micron, are included. Among these are calcium aluminum silicate, calcium sodium silicate, potassium silicate, aluminum silicate, calcium zinc silicate, and the like. Magnesium silicates, strontium silicates and barium silicates possessing the above enumerated physical and chemical characteristics are likewise of utility.

Finely divided, amorphous, precipitated pigmentary silica can be employed. Usually these silicas are of from 20 to 120 square meters per gram BET surface area and have ultimate particle sizes on the order of those of the described calcium silicates, e.g. below 1.0 micron and notably less than 0.3 micron. They too are composed of flocs of ultimate particles.

The preferred siliceous materials contain both "bound water" and "free water." "Free water" is that water which is removed by heating for 24 hours at 105° C.

"Bound water" is the difference between the "free water" and that water which is removed by heating at ignition temperatures, e.g. 1000 to 1200° C. It appears the "bound water" is chemically united, whereas the "free water" is more loosely contained by the siliceous material.

The titanium dioxide component is comprised of the usual paper pigment quality titanium dioxide, e.g. a finely divided, particulate material having particles on the average of 0.3 micron diameter. Other grades of pigmenting titanium dioxide may find utility, especially in view of the beneficiating effect of the siliceous material.

The following examples illustrate the manner in which this invention may be practiced:

#### EXAMPLE I

A pulp beater was charged with 250 grams of kraft pulp and 250 grams of sulfite pulp, dispersed in 23 liters of water and beaten in a Niagara beater to a freeness of 550 milliliters (Canadian standard). To this beaten pulp was added 400 cubic centimeters of aqueous slurry containing 35 grams of pigment comprised of titanium dioxide and/or calcium silicate, as indicated in Table I, followed by mixing for five minutes. A small quantity of aluminum sulphate octadecahydrate, as indicated in Table I, was added adjusting the slurry pH at 5.0. The resulting acidic slurry was then sheeted on a laboratory Noble-Wood sheeting machine and the opacity, brightness and ash content of the paper determined.

The titanium dioxide charged comprised paper grade material and had an average particle size of 0.3 micron. The calcium silicate used had a BET surface area of 31 square meters per gram, and an average ultimate particle size of 0.04 to 0.08, with particles ranging from 0.015 to 0.20 micron. By chemical analysis it was comprised of 66.4 percent  $\text{SiO}_2$ , 18.6 percent  $\text{CaO}$ , 0.39 percent Na and 0.60 percent chlorine. In aqueous slurry it had a pH of 10.6. Upon heating at ignition temperature 1000° C., it lost 15.1 percent by weight, and upon heating at 105° C. in a laboratory drier for 24 hours it lost 5.2 percent by weight, indicating a free water content of 5.2 percent and a bound water content of 9.9 percent by weight.

Table I lists the various reaction variables along with the properties of the prepared paper.

Table I

| Loading-Weight, Percent <sup>1</sup> | Paper Properties |                |                   |                     |                  |
|--------------------------------------|------------------|----------------|-------------------|---------------------|------------------|
|                                      | Calcium Silicate | $\text{TiO}_2$ | Alum <sup>2</sup> | Ash, Weight Percent | Opacity, Percent |
| 0                                    | 10               | 0.3            | 6.57              | 86.4                | 85.9             |
| 2                                    | 8                | 1.7            | 8.31              | 88.5                | 86.7             |
| 4                                    | 6                | 3.1            | 7.95              | 88.1                | 86.7             |
| 6                                    | 4                | 4.6            | 7.50              | 86.9                | 85.7             |
| 8                                    | 2                | 6.0            | 6.85              | 84.6                | 84.7             |
| 10                                   | 0                | 7.5            | 6.66              | 81.4                | 82.2             |

<sup>1</sup> Total pigment loading is 10 percent by weight.

<sup>2</sup> Weight percent, based on dry pulp, of  $\text{Al}_2(\text{SO}_4)_3 \cdot 18\text{H}_2\text{O}$ .

Figure 1 of the drawings graphically correlates the variations in ash and opacity of the paper as it was effected by changes in the pigment composition. The unusual results of increased opacity and pigment retention (as denoted by ash contents), along with brightness (not included in the graph) emphasizes the unique synergistic coaction herein obtained.

#### EXAMPLE II

Following the procedure of Example I, with the exception that the pulp charge of 500 grams consisted of air dried bleached kraft pulp which was beaten to 400 milliliters' freeness paper was prepared. Table II, hereafter, lists the experimental variables and properties of the resulting papers.

5  
Table II

| Loading-Weight, Percent <sup>1</sup> |                  |                   | Paper Properties    |                  |                     |
|--------------------------------------|------------------|-------------------|---------------------|------------------|---------------------|
| Calcium Silicate                     | TiO <sub>2</sub> | Alum <sup>2</sup> | Ash, Weight Percent | Opacity, Percent | Brightness, Percent |
| 0                                    | 10               | 0.3               | 4.3                 | 81.1             | 81.7                |
| 2                                    | 8                | 1.7               | 8.1                 | 87.3             | 85.4                |
| 4                                    | 6                | 3.2               | 7.8                 | 87.9             | 84.1                |
| 6                                    | 4                | 4.6               | 7.7                 | 86.5             | 85.0                |
| 8                                    | 2                | 6.0               | 7.3                 | 84.3             | 84.2                |
| 10                                   | 0                | 7.4               | 7.2                 | 81.1             | 81.2                |

<sup>1</sup> Total pigment loading is 10 percent by weight.<sup>2</sup> Weight percent, based on dry pulp, of Al<sub>2</sub>(SO<sub>4</sub>)<sub>3</sub>·18H<sub>2</sub>O.

Figure 2 of the drawings graphically shows the variations in paper opacity observed as the pigment components were varied. It will be noted that whenever the pigment comprised both titanium dioxide and calcium silicate, the paper opacity exceeded the opacity of paper pigmented individually with each component. A substantial improvement in opacity is observed over a wide range of mixtures.

## EXAMPLE III

A pulp beater was charged as follows:

|                              | Grams |
|------------------------------|-------|
| Unbleached sulfite pulp      | 90    |
| Bleached kraft pulp          | 180   |
| Hard white envelope cuttings | 90    |

This charge was dispersed in 23 liters of water and the resulting slurry was beaten in a Niagara beater for about 80 minutes to approximately 400 milliliters' freeness, Canadian standard (TAPPI Standard T227 m 50). One hundred milliliters of prepared rosin of about 5 percent by weight size was then added. Thereafter, 9 grams of pregelatinized starch was added and the pulp was circulated in the beater long enough to insure complete mixing. Aluminum sulphate in the amount of 3 percent by weight, based on the dry weight of pulp, was added as a solution containing 12.92 grams of aluminum sulphate octadecahydrate per liter. At this stage, the pulp consistency was approximately 1.1 percent. Stirring was continued for 2 minutes. Immediately thereafter, the amounts of calcium silicate having the composition CaO(SiO<sub>2</sub>)<sub>3.3</sub> and titanium dioxide indicated in the table were added. The amounts are expressed as percentages of the dry weight of the pulp. Stirring of the mixture was continued for 10 minutes more, and the resulting stock was diluted to 8,000 milliliters, divided into ten 800-milliliter portions, and sheeted into paper. The paper was tested for brightness, opacity, bursting strength, weight and thickness, and ash and moisture content, with the following results:

Table III

|                                         | 1    | 2    |
|-----------------------------------------|------|------|
| Percent titanium dioxide by weight      | 1.0  | 0.5  |
| Percent calcium silicate by weight      | 1.0  | 2.5  |
| Brightness:                             |      |      |
| Green light                             | 70.8 | 70.0 |
| Blue light                              | 61.2 | 62.2 |
| Contrast ratio (green light):           |      |      |
| Reflectance, black backing              | 56.9 | 57.0 |
| Reflectance, white backing              | 79.0 | 80.1 |
| Ratio                                   | 72.1 | 71.2 |
| Contrast ratio (blue light):            |      |      |
| Reflectance, black backing              | 53.7 | 53.9 |
| Reflectance, white backing              | 66.8 | 67.9 |
| Ratio                                   | 76.2 | 75.3 |
| Bursting strength, lb./in. <sup>2</sup> | 32.0 | 34.5 |
| Percent ash in oven dry paper           | 2.28 | 2.63 |

Pulp slurries from which paper is sheeted are usually prepared by beating in regular fashion any type of acceptable cellulosic pulp, e.g. sulfite pulp, soda or kraft pulp, semi-commercial pulp, mechanically ground pulp and mixture of one or more of such pulps. Besides virgin pulp, broke, i.e. cuttings and paper scraps recovered from

## 6

prior paper making operations can be included. From 3 to 6 percent by weight of the slurry is pulp (dry basis) in accordance with normal operations.

- Sufficient pigments are added to constitute from 0.5 to 30 percent by weight of the pulp on a dry basis. Ash values of the paper, by virtue of the high pigment retention obtained hereby, range from about 50 to 80 or 90 percent of the pigment concentration in the slurry on a dry pulp basis.
- 10 In practicing paper pigmentation according to this invention, other paper making operations may be included. Sized or unsized paper can be prepared. For sized paper, a rosin size such as a soluble alkali metal rosin soap, e.g. sodium resinate or other typical size is included in the pulp slurry and precipitated by use of a trivalent or tetravalent metal such as titanic sulphate or aluminum sulphate.

- 15 Coloring matter, if desired, can be included in the pulp slurry during the beating cycle. Also, the pulp may be bleached by treatment with chlorine in an oxidizing form or with other bleaching agents.

- 20 Subsequent to sheet formation, the sheet is suitably dried and, when necessary, calendered. Coatings may be applied to the sheet in the preparation of high grade printing papers of the type used in more expensive magazines. A typical coating agent is finely divided clay.

- 25 This application is a continuation of application Serial No. 543,835, filed October 31, 1955, now abandoned, which is a continuation-in-part of prior applications Serial Nos. 352,295, now abandoned, and 393,522, filed respectively on April 30, 1953 and November 20, 1953.

- 30 Although the present invention is described with reference to particular details of special embodiments, it is not intended that it be limited thereto except insofar as 35 the invention is defined in the claims.

I claim:

1. The method of preparing paper of enhanced opacity which comprises adding titanium dioxide and a flocculent finely divided, pigmentary, amorphous, precipitated 40 siliceous material having an average ultimate particle size below 1.0 micron in an aqueous paper pulp slurry, adjusting the pH of such slurry to between 4 and 6.5 by inclusion in the aqueous pulp slurry of an acidic material prior to sheeting and sheeting the slurry.

- 45 2. The method of preparing paper of enhanced opacity which comprises adding titanium dioxide and a flocculent finely divided, pigmentary, amorphous, precipitated alkaline earth metal silicate having an average ultimate particle size below 1.0 micron in an aqueous pulp slurry, 50 adjusting the pH of said slurry to between 4 and 6.5 by inclusion in the aqueous pulp slurry prior to sheeting an acidic material which forms a water insoluble alkaline earth metal salt and sheeting the slurry.

3. The method of preparing paper of enhanced opacity 55 which comprises adding titanium dioxide and a flocculent finely divided, pigmentary, amorphous, precipitated calcium silicate having an average ultimate particle size below 1.0 micron in an aqueous pulp slurry, adjusting the pH of said slurry to between 4 and 6.5 by inclusion 60 in the aqueous pulp slurry prior to sheeting an acidic material which forms a water insoluble calcium salt and sheeting the slurry.

4. The method of preparing paper of enhanced opacity which comprises adding titanium dioxide and flocculent 65 finely divided, pigmentary, amorphous, precipitated calcium silicate having an average ultimate particle size below 1.0 micron in an aqueous pulp slurry, adjusting the pH of such slurry to between 4 and 6.5 by inclusion 70 in the aqueous pulp slurry of aluminum sulphate prior to sheeting, and sheeting the slurry.

5. The method of claim 4 wherein the calcium silicate corresponds to the formula, CaO(SiO<sub>2</sub>)<sub>x</sub>, x ranging from 2 to 5.

6. The method of claim 4 wherein the calcium silicate 75 corresponds to the formula, CaO(SiO<sub>2</sub>)<sub>x</sub>, x ranging from

2 to 5, has a surface area of 10 to 200 square meters per gram and is of below 1.0 micron in average ultimate particle size.

7. Pigmented cellulosic paper of enhanced opacity pigmented with independently prepared titanium dioxide and a flocculent finely divided, pigmentary, amorphous, precipitated siliceous material having an average ultimate particle size below 1.0 micron and containing at least 50 percent  $\text{SiO}_2$  by weight.

8. Pigmented cellulosic paper of enhanced opacity containing independently prepared titanium dioxide and a flocculent finely divided, pigmentary, amorphous, precipitated siliceous material having an average ultimate particle size below 1.0 micron and of at least 50 percent  $\text{SiO}_2$  content by weight, the titanium dioxide constituting from 10 to 95 percent by weight thereof and the siliceous material.

9. Pigmented cellulosic paper of enhanced opacity containing independently prepared titanium dioxide and a flocculent finely divided, pigmentary, amorphous, precipitated siliceous material having an average ultimate particle size below 1.0 micron and of at least 50 percent  $\text{SiO}_2$  content by weight, the titanium dioxide constituting from 35 to 95 percent by weight thereof and the siliceous material.

10. Pigmented cellulosic paper of enhanced opacity containing as opacity enhancing components flocculent finely divided, amorphous, precipitated siliceous pigmentary material containing at least 50 percent  $\text{SiO}_2$  by weight and having an average ultimate particle size of less than 1 micron and titanium dioxide, said titanium dioxide constituting from 35 to 95 percent by weight of the titanium dioxide and said siliceous material, the opacity of said paper being greater than that of paper containing as its opacity enhancing component titanium dioxide in an amount equal to that of the siliceous material and titanium dioxide in the paper.

5

15

20

30

35

11. A paper pigment composition effective in enhancing the opacity of cellulosic paper containing as opacity enhancing components flocculent finely divided, amorphous, precipitated siliceous pigmentary material containing at least 50 percent  $\text{SiO}_2$  by weight and having an average ultimate particle size of less than 1 micron and titanium dioxide, said titanium dioxide constituting 10 to 95 percent by weight of the titanium dioxide and siliceous material.

12. A paper pigment composition effective in enhancing the opacity of cellulosic paper containing as opacity enhancing components independently prepared, flocculent finely divided, amorphous, precipitated siliceous pigmentary material containing at least 50 percent  $\text{SiO}_2$  by weight and having an average ultimate particle size of less than 1 micron and titanium dioxide, said titanium dioxide constituting 35 to 95 percent by weight of the titanium dioxide and siliceous material, said pigment being capable of enhancing the opacity of cellulosic paper to a greater degree than the same amount of titanium dioxide without the siliceous material.

13. A paper pigment composition effective in enhancing the opacity of cellulosic paper containing as opacity enhancing components flocculent finely divided precipitated siliceous pigmentary material containing at least 50 percent  $\text{SiO}_2$  by weight and having an average ultimate particle size of less than 0.3 micron and titanium dioxide, said titanium dioxide constituting 35 to 95 percent by weight of the titanium dioxide and siliceous material.

## References Cited in the file of this patent

## UNITED STATES PATENTS

|           |           |               |
|-----------|-----------|---------------|
| 2,000,031 | Larson    | May 7, 1935   |
| 2,378,193 | Cummins   | June 12, 1945 |
| 2,739,068 | Eichmeier | Mar. 20, 1956 |
| 2,786,757 | Taylor    | Mar. 26, 1957 |
| 2,786,777 | Allen     | Mar. 26, 1957 |

UNITED STATES PATENT OFFICE  
CERTIFICATION OF CORRECTION

Patent No. 2,943,971

July 5, 1960

Louis B. Taylor

It is hereby certified that error appears in the above numbered patent requiring correction and that the said Letters Patent should read as corrected below.

Column 3, lines 37 and 38, for "beneficating" read  
-- ~~beneficiating~~ --; column 5, Table III, first column, line  
14 thereof, for "Bursting strength, lb./in<sup>2</sup>" read -- ~~Bursting~~  
~~strength, lb./in.~~<sup>2</sup> --; column 6, line 47, for "finely" read  
-- ~~finely~~ --; column 8, line 14, for "containig" read  
-- ~~containing~~ --.

Signed and sealed this 25th day of July 1961.

(SEAL)

Attest:

ERNEST W. SWIDER

Attesting Officer

DAVID L. LADD

Commissioner of Patents